

# UNITED STATES PATENT OFFICE.

CHARLES A. HANSEN, OF SCHENECTADY, NEW YORK, ASSIGNOR TO GENERAL ELECTRIC COMPANY, A CORPORATION OF NEW YORK.

## INCANDESCENT-LAMP FILAMENT.

1,026,392.

Specification of Letters Patent.

Patented May 14, 1912.

No Drawing.

Application filed April 8, 1908. Serial No. 425,814.

To all whom it may concern:

Be it known that I, CHARLES A. HANSEN, a citizen of the United States, residing at Schenectady, county of Schenectady, State 5 of New York, have invented certain new and useful Improvements in Incandescent-Lamp Filaments, of which the following is a specification.

In the production of incandescent lamp 10 filaments consisting of tungsten, titanium, zirconium, and similar refractory metals and compounds, it has been customary to use some sort of a binding material by the aid of which the powdered refractory metal 15 or material could be shaped into threads or wires. Some inventors have made use of carbonaceous binders, such as tragacanth, sugar solutions, glucose, and starch paste, but the removal of the carbonaceous residue 20 left by such binders has, in general, proved difficult and expensive.

According to my present invention, refractory powdered material, such as tungsten, is shaped into threads or wires by means 25 of a binder which on a further treatment breaks up or decomposes, and furthermore is of such a nature and breaks up in such a way that the residue is not injurious to the filament and need not be removed there- 30 from. In fact, the particular binder herein- after mentioned as a specific embodiment of my invention yields a residue of such low conductivity that the completed filament has a high specific resistance and can be used 35 on relatively high voltages.

The binders contemplated by my present invention include those sticky metal oxalates which when highly heated calcine to a stable and refractory oxid of the metal. 40 Zirconium oxalate is typical of this class. Its use in the production of filaments consisting essentially of tungsten is hereinafter described in detail, and will serve to give persons skilled in the art a working knowl- 45 edge of my invention.

Zirconium oxalate can be prepared by precipitation of hot zirconium nitrate solution with ammonium oxalate. The precipitate is gelatinous in character, resembling starch 50 paste in consistency, and has a smooth, even texture. By using ordinary care during manufacture, the zirconium oxalate can be made exceedingly pure.

In making up the mixture of powdered

tungsten and zirconium oxalate, I may use 55 just sufficient oxalate to give tenacity to the mass, or I may use a much greater quantity with the idea of thereby obtaining a filament of particularly high specific resistance.

The plastic mass above described can be 60 squirted into wires or threads in an ordinary manner and should then be dried and finally heated to a high temperature to calcine the oxalate and convert it into zirconium oxid. This high temperature treatment 65 may be effected by passing current through the filament while supported in a vacuum or suitable gas, the heat treatment being carried far enough to completely sinter and shrink the filaments into a coherent and 70 homogeneous body of tungsten uniformly mixed with zirconium oxid.

As an alternative method of heating, I may make use of the vacuum furnace shown 75 in United States Patent to Arsen #785,535, March 21, 1905, though I prefer to use in place of the graphite heater there shown a heater consisting entirely of tungsten. If desired, the heat treatment in the furnace may be stopped somewhat short of complete 80 shrinkage, thus permitting completion and shaping of the filaments in treating bottles or in the lamp bulbs themselves.

What I claim as new and desire to secure by Letters Patent of the United States, is— 85

1. The method of filament manufacture which consists in forming threads consisting of a mixture of powdered refractory conductive material with a binder composed essentially of a gelatinous oxalate of a metal having 90 a stable refractory oxid, and subsequently heating said threads to convert the oxalate into the oxid and to consolidate the materials into a coherent conductor.

2. The method of filament manufacture 95 which consists in forming threads consisting of refractory metal powder held together by a binder composed essentially of a gelatinous oxalate decomposable to yield a refractory oxid, and heating said threads in an inert environment to convert the oxalate into 100 oxid and to consolidate and sinter the refractory metal.

3. The method of filament manufacture 105 which consists in forming threads consisting of refractory powder held together by a binder composed essentially of zirconium oxalate, and subsequently treating these

threads to convert them into homogeneous conductors containing zirconium oxid mixed with refractory material.

4. The method of filament manufacture which consists in forming threads consisting of tungsten powder with a binder composed essentially of zirconium oxalate, and subsequently treating said threads to convert them into homogeneous conductors containing zirconium oxid mixed with refractory oxid.

5. A squirting mixture for the production of lamp filaments, consisting of powdered refractory material and a binder composed essentially of a metal oxalate decomposable to produce a stable refractory oxid.

6. A squirting mixture for lamp filaments

consisting of powdered refractory material and a binder composed essentially of zirconium oxalate.

7. A squirting mixture for lamp filaments consisting of tungsten powder and a binder composed essentially of zirconium oxalate.

8. A squirting mixture for lamp filaments consisting of tungsten powder and a binder composed essentially of an oxalate decomposable to yield a stable refractory oxid.

In witness whereof I have hereunto set my hand this 7th day of April, 1908.

CHARLES A. HANSEN.

Witnesses:

HELEN ORFORD,  
BENJAMIN B. HULL.